

# UNITED STATES PATENT OFFICE.

ALADAR PACZ, OF CLEVELAND HEIGHTS, OHIO.

## ALLOY.

1,387,900.

Specification of Letters Patent. Patented Aug. 16, 1921.

No Drawing.

Application filed February 13, 1920. Serial No. 358,555.

To all whom it may concern:

Be it known that I, ALADAR PACZ, a citizen of the United States, residing at Cleveland Heights, in the county of Cuyahoga and State of Ohio, have invented a certain new and useful Improvement in Alloys, of which the following is a full, clear, and exact description.

This invention relates to alloys and has 10 for its general object the provision of a metallic composition which shall possess a smaller unit weight for a given amount of strength than alloys heretofore known and used commercially.

15 In the making of crank cases and pistons for internal combustion motors, of disk wheels, floor plates and running boards for vehicles, casings for suction cleaners, culinary utensils, machine parts and patterns 20 and a great many other purposes, it is desirable to employ a casting metal of considerable rigidity and very light weight, one of the requirements being that the metal shall be susceptible of easy machining. One 25 of the best known and most used of these alloys has been that known as "No. 12 metal" which consists approximately of aluminum 92, copper 8, sometimes with a very small addition of iron. This metal ordinarily possesses tensile strength of from 17,000 to 30 18,000 pounds per square inch with an elongation of from one to one and one-half per cent., and with present prices of ingredients (aluminum 33¢ and copper 20¢ per pound) 35 costs about \$640.00 per ton.

The objects of my invention are the provision of a metal which shall cast fully as well as any aluminum alloy heretofore known; which shall have a lower coefficient 40 of heat expansion than other aluminum alloys and hence shrink less on cooling; which shall have a higher tensile strength and a higher elongation than any known aluminum alloy of equal density; which shall be 45 as easily machined, and shall be lower in price; which shall yield perfect castings throughout a wide range of pouring temperatures; while further objects and advantages of my invention will become apparent 50 as the description proceeds.

My improved composition is characterized by containing upward of 80% of aluminum combined with at least about 5% of silicon, with or without small additional quantities 55 of other metals, such for example as a small

amount of iron, but those other metals preferably constituting not over about 2% of the whole. The presence or absence of the last named metals is not considered as bearing upon my invention, which derives 60 its principal characteristics from the combination of aluminum with the comparatively large amount of silicon mentioned; and the preferred species is that containing aluminum and silicon in the proportion of 65 approximately seven to one regardless of the presence or absence of small quantities of additional elements, although any composition containing between 8% and 15% of silicon lies within a very valuable range. 70 It has heretofore been supposed that the largest amount of silicon which could be incorporated with aluminum was about one half of one per cent., and I am able to secure the assimilation of this comparatively 75 large quantity only by the employment of a grain-refining process certain of which I will now describe.

I preferably produce my improved alloy by melting together commercial aluminum 80 and commercial metallic silicon, consisting ordinarily of about 90% pure silicon together with about 10% of impurities, the chief of which are silica, carborundum, iron silicid, calcium silicid, aluminum, and iron. 85 According to my preferred procedure I first melt together 1 part of this material with 4 parts of aluminum in a suitable crucible and after the batch has become thoroughly melted, decant the same either into another 90 crucible or into suitable ingot molds, this being for the purpose of removing the non-metallic impurities which become incrusted upon the interior of the crucible. I then add further aluminum to this mixture in 95 any proportion from about 25% to 50%; if less than about 25% of additional aluminum be employed, the resulting alloy becomes increasingly brittle and above about 50% of additional aluminum, the resulting alloy becomes 100 increasingly soft, although I do not restrict myself exactly to these limits inasmuch as there are some uses for which the same can be exceeded without danger. I preferably employ about 33% of added alu- 105 minum to 66% of the first mixture, whereby there is produced the preferred composition first mentioned, namely aluminum 7, silicon 1. It is equally within my invention and produces the same ultimate alloy to melt the 110

ingredients directly together in the final proportion desired, but the same is less convenient practically because of the larger quantity of material necessary to handle 5 during the refining operation.

The resulting alloy if cast directly has a very coarse, dark, crystalline fracture and its physical properties are quite low, the tensile strength running from about 15,000 to 10 18,000 pounds per square inch with an elongation of from one-half per cent. to one and one-fourth per cent. However, before casting this metal into the finished form, I treat it at a temperature above its melting 15 point with an alkaline fluorid or a combination of fluorids, one at least of which is that of an alkali: for example, sodium fluorid, potassium fluorid or lithium fluorid either alone or mixed with calcium fluorid, barium 20 fluorid, strontium fluorid or magnesium fluorid. I preferably employ sodium fluorid as a base and use at least about one per cent. of the same by stirring the pulverized compound into the molten metal with a carbon 25 rod, whereupon a yellow flame appears suggestive of the combustion of metallic sodium, accompanied by a dense, acrid, white smoke. This stirring is continued rather briskly until the evolution of flame 30 and smoke ceases. If now the metal be cast, it will be found that the fracture instead of being coarse, dark, and glassy, is fine-grained, light and dense. The physical properties have undergone a most remarkable 35 change, the tensile strength rising to a point between 23,000 and 27,800 pounds per square inch and the elongation to a point between  $3\frac{1}{2}\%$  to  $6\frac{1}{4}\%$ . Accordingly the composition is stronger than any commercial 40 casting alloy of equal density, being fully ten per cent. lighter than the "Number 12 metal" heretofore mentioned and at the present prices of ingredients (silicon 13¢ per pound) costs only \$600.00 per ton as 45 against \$640.00 for "Number 12 metal." Compared by volume with "Number 12 metal" my alloy is the cheaper in the proportion of 6 to 7 and upon the basis of the tensile strength my improved composition is 50 superior to Number 12 metal in the proportion of 6 to 9. The castings run freely, expand sufficiently on solidification to copy the mold with great exactness, shrink on cooling less than any other known aluminum 55 alloy, are free from blow-holes or pin-holes, can be readily machined, and take and retain a high polish. My alloy is also excellent for die castings, and after the alkali fluorid treatment herein described it can be 60 forged and drawn into wire and possesses considerable ductility when cold.

Furthermore these successful castings can be secured without any special care as to temperatures, which is a very important 65 feature in commercial foundry practice.

I do not confine myself to any one source of silicon; I do not exclude the use of additional metallic ingredients so long as the amounts of silicon and aluminum are retained within the relative proportions herein mentioned; I do not restrict myself to the addition of an alkaline fluorid only in the precombined state since I have had excellent results by using a mixture of sodium chlorid and calcium fluorid and I conceive 70 that other fluorid compounds can be employed; and I do not limit myself to any theory of operation but only set forth herein in the results of my actual observations and discoveries, restricting myself to details only 75 as specifically recited in the claims hereto annexed. The present application is limited to the alloying and treatment of alloys containing aluminum and silicon, the more general idea of refining metals and alloys by 80 treatment with compounds containing fluorin and alkali being set forth and claimed in my companion application filed May 11, 1921, Serial No. 468,778.

Having thus described my invention, what 90 I claim is:

1. A casting alloy capable of being machined containing between about 8 per cent. and about 20 per cent. of silicon and at least about 98 per cent. of the balance being aluminum. 95

2. A casting alloy capable of being machined containing between 8 per cent. and 15 per cent. of silicon and the balance mostly aluminum. 100

3. A casting alloy capable of being machined and consisting mostly of aluminum and silicon, said alloy containing substantially one part of silicon to eight parts of aluminum. 105

4. A casting alloy capable of being machined containing at least 80 per cent. of aluminum, combined with at least 8 per cent. of silicon. 110

5. A fine grained, tenacious, machinable alloy made mostly of commercial aluminum and commercial silicon and containing not more than about 2 per cent. of any metal having an atomic weight above 60. 115

6. The process of treating alloys of aluminum and silicon which contains the step of stirring an alkaline fluorid into the molten mass. 120

7. The process of producing an alloy of aluminum and silicon, wherein the latter constitutes at least about 8 per cent. of the whole which contains the step of stirring into the molten mass at least about  $1\frac{1}{2}$  per cent. of an alkaline fluorid. 125

8. The process of producing an alloy of aluminum and silicon wherein the latter constitutes at least about 8 per cent. of the whole which contains the steps of first melting together commercial aluminum and commercial silicon, decanting the molten mass to 130

remove non-metallic impurities and subsequently incorporating in the molten mass a quantity of alkali fluorid.

9. The process of producing an alloy of 5 aluminum and silicon which contains the steps of melting together about 4 parts of commercial aluminum and 1 part of commercial silicon, pouring the mixture, adding more aluminum in the proportion of 10 from one to three parts of such mixture to each part of aluminum added, and thereafter incorporating with the molten mass at least about 1 per cent of an alkali fluorid.
10. The process of disseminating silicon 15 in aluminum which consists in subjecting the molten ingredients to the action of an alkali fluorin compound.
11. The process of disseminating upward

of 5 per cent. of silicon throughout aluminum to produce a fine grained ductile alloy 20 which consists in subjecting the molten ingredients to the action of one or more other compounds which contain fluorin and an alkali.

12. An alloy of aluminum and silicon 25 which contains between 8 per cent. and 20 per cent. of silicon and whose elongation is at least 3 per cent.

13. An alloy of aluminum containing upward of 8 per cent. silicon having a specific 30 gravity less than 2.7, a tensile strength upward of 23,000 pounds per square inch, and an elongation upward of 3 per cent.

In testimony whereof, I hereunto affix my signature.

ALADAR PACZ.